

Dec. 14, 1926.

1,610,567

H. S. MARSH ET AL

ANNEALING OF SHEET STEEL

Filed Oct. 7, 1925

2 Sheets-Sheet 1



FIG. I.

WITNESSES

J. Hark Bradley  
Percy A. Englin

INVENTORS  
Henry S. Marsh  
Ralf S. Cochran  
by Chrity and Chrity  
their attorneys

Dec. 14, 1926.

1,610,567

H. S. MARSH ET AL

ANNEALING OF SHEET STEEL

Filed Oct. 7, 1925

2 Sheets-Sheet 2



FIG. II.

WITNESSES  
Percy A. Englich  
Mary A. Wall

INVENTORS

Henry S. Marsh  
Raef S. Coelran  
My Chrity and Chrity  
their attorneys

## UNITED STATES PATENT OFFICE.

HENRY S. MARSH AND RALF S. COCHRAN, OF YOUNGSTOWN, OHIO.

## ANNEALING OF SHEET STEEL.

Application filed October 7, 1925. Serial No. 60,978.

Our invention relates to the annealing of sheet steel and consists in a method whereby relatively high ductility but within properly controlled limits, is attained.

In the practice of our invention we conveniently employ a continuous furnace, whose structure and mode of operation will be sufficiently understood by reference to the accompanying drawings. Fig. I shows the furnace in horizontal section, and Fig. II shows it in vertical and medial section.

Steel sheets are generally rolled at such low temperature, that the crystals or "grains" are badly distorted, and consequently it becomes necessary to anneal the sheets after they have been rolled, in order to restore the normal grain structure, and render the sheets suitable for the drawing operations which at the present day are widely practiced. Some years ago rolled steel sheets were ordinarily "box" annealed. But box annealing gives widely varying results; sometimes the annealed sheets are very stiff, and sometimes they are of "leaden" softness, and the product which approaches either of these extremes is unsuitable for the drawing trade. A later practice has been to "blue" anneal sheets which are intended to be used in drawing operations, and sometimes to box anneal afterwards. But still the results are erratic and not to be depended on: box annealing causes "grain growth," and sheets which are blue annealed are subject to scaling. The consequent roughness of surface cannot be entirely eliminated in subsequent cold rolling.

Such, however, are the limitations under which the art has progressed hitherto; and the trade is constantly demanding of the steel maker better and better sheets. Our process overcomes these limitations.

We first heat the rolled sheet material in a non-oxidizing atmosphere to the requisite high temperature, which for ordinary commercial steels is from 1750° to 1800° F., preferably to the higher figure; and then, while still maintaining the non-oxidizing atmosphere, we cool it again through a range of 200° to 300° downward from the maximum, indicated. Having accomplished this,

we allow the cooling to proceed with no further concern to maintain a non-oxidizing atmosphere, and preferably in the open air, until the material comes to a dull red heat. At this temperature we pass the sheets through a roller leveler, which flattens them, and incidentally cools them through another hundred degrees, more or less. We then make the sheets up into packs of from three to six inches thick; they are then of just visible redness. And we then set the packs aside to cool to atmospheric temperature.

The initial steps of heating and cooling in a non-oxidizing atmosphere may be carried out in a continuous furnace of the ordinary open type, modified to serve the ends described. Through the furnace shown in the drawings the sheets advance from left to right. The furnace toward the intake end is provided with burners 1, through which flame has ingress, and in the proper operation of the furnace the flame will be of non-oxidizing character, or substantially so, and under ordinary conditions of operation such ingress of air as occurs still leaves the atmosphere within the furnace substantially neutral. The furnace stack 2 is to the right, and the flow of flame and hot gases is in the direction of the advance of the material, from left to right.

The furnace is made much longer than such furnaces ordinarily are, and toward the delivery end there is no inflow of flame. Toward the delivery end accordingly the stream of gases, non-oxidizing in character, is cooling and the advancing sheets are giving up their heat and becoming cooler.

Furnace structure and operation will vary in detail, to suit the character of the material which is habitually or occasionally run through it. For instance, when thick sheets are being annealed at high speed, relatively large quantities of heat are given up to and absorbed by the walls at the cold end of the furnace. To meet such a condition, the furnace walls may be made thin, and pipes of familiar construction may be provided within the furnace walls, for the circulation of water, to carry away the excess heat, perhaps regularly, perhaps when specially re-

quired. With like ends in view, a bridge wall, such as is indicated at 3, Fig. II, may be provided within the furnace, to absorb and reflect heat, and render the cold end 5 of the furnace cooler, while operation progresses.

Temperature conditions within the furnace may be observed by means of a radiation pyrometer, and furnace operation 10 controlled accordingly.

Typically we so proportion the parts of the apparatus which we employ, and we drive our conveyer at such speed, that the steps of our operation proceed as follows: 15 heating quickly, within an interval of from 2 to 7 minutes in a nearly neutral atmosphere, to a temperature of 1700° to 1850° F.; cooling quickly, within an interval of from 1/2 minute to 2 minutes, and still in a nearly 20 neutral atmosphere, to a temperature of 1200° to 1400° F.; continued cooling quickly (and conveniently in the open air) in about 1 to 2 minutes, to dull red; roller leveling; 25 then cooling slowly in 1 to 3 hours, in packs, in the open air, to a temperature of 200° F. or less.

After performing the annealing operation described, the sheet ordinarily is pickled before use.

30 Certain details remain to be more particularly mentioned. Variations in sheet thickness are in ordinary practice substantially offset by varying accordingly the number of sheets which are caused to pass at once 35 through the furnace. When we anneal 11-gauge sheets, we pass them through, one at a time. We ordinarily pass 16-gauge sheets through, two at a time; and 20-gauge, three 40 at a time. Finer adjustment may be effected by varying the speed of the conveyor. Thin sheets, if run singly, would heat too rapidly and would chill before they could be made up in packs. The cooler the sheets 45 when made up in packs, the thicker the packs can be made, without too much softening.

When making up the pack, the first sheet alone tends to cool rapidly, but the superposition of successive sheets arrests the fall 50 of temperature and undue chilling is prevented. The 6-inch pack is the practical optimum. The more sheets in a pack, the fewer lifts of the crane required for setting them aside to cool; but, in a 12-inch pack, 55 for instance, cooling proceeds so slowly that the sheets tend ultimately to be softer than we desire them to be. The outermost sheets are, of course, always cooler than those within the pack, but there is a permissible range 60 within which the cooling step may proceed. And we have found, all things considered, that a 6-inch pack is best.

Our invention may be practiced with 65 some refinement in detail, to produce a sheet of still better drawing quality, in case the

use required of it can justify the somewhat greater cost. In this case the furnace is made very tight, in order to keep out all air, and a completely reducing atmosphere is maintained within the furnace. And 70 protection in a reducing atmosphere may be prolonged to the non-tarnishing degree of approximately 400° F. In this case cooling will preferably be so controlled as to be achieved in five to ten minutes. The 75 sequence in treatment then is: hot roll, roller level, pickle, cold roll, anneal. In this case, it will be observed, pickling after annealing is not required. Pickling as a last operation (particularly when the sheets are 80 immediately to be put on the drawing press, as when the customer does the pickling) sometimes renders the metal brittle. Heating removes such brittleness, supposedly by driving out occluded hydrogen. Another 85 reason why ultimate pickling is advantageously avoided, is that when the sheet is under the drawing operation subjected to tensile stress, small surface depressions, such as are incident to pickling, tend to weaken 90 the metal irregularly. Again, a smooth sheet will during the drawing operation slip over the corner of the die with less resistance than a rough one, and in that respect the 95 danger of a break in the sheet is diminished. From this it is clear that a smooth sheet, annealed after cold rolling, is better than a rough sheet, pickled after annealing. Such is our preferred procedure, when the customer's job is such as to warrant the extra 100 expense of cold rolling, and the maintenance of a furnace with air-tight walls.

We claim as our invention:

1. The method herein described of annealing sheet steel which consists in heating the 105 sheet material in a non-oxidizing atmosphere to a temperature of 1750° F. as a minimum, cooling the material while maintaining it still in a non-oxidizing atmosphere to a temperature of 1550° F. as a maximum, 110 cooling it thence to a dull red in the open air, making the material at the temperature last indicated into packs, and allowing the 115 packs to cool in the air to atmospheric temperature.

2. The method herein described of annealing sheet steel which consists in heating the sheet material within a maximum time interval of seven minutes and while maintained in a non-oxidizing atmosphere to a 120 temperature of 1750° F. as a minimum, cooling the material within a maximum interval of two minutes and while still maintained in a non-oxidizing atmosphere to a temperature of 1550° F. as a maximum, and then 125 completing the cooling in the open air.

3. The method herein described of annealing sheet steel which consists in heating the sheet material within a maximum time interval of seven minutes and while main- 130

tained in a non-oxidizing atmosphere to annealing temperature, cooling the material within a maximum interval of two minutes and while still maintained in a non-oxidizing atmosphere to a temperature of 1550° F. as a maximum, cooling it further and within a maximum time interval of two minutes to dull red, then making the material into packs, and allowing the packs to cool in the air to atmospheric temperature. <sup>10</sup>

In testimony whereof we have hereunto set our hands.

HENRY S. MARSH.  
RALF S. COCHRAN.

tained in a non-oxidizing atmosphere to annealing temperature, cooling the material within a maximum interval of two minutes and while still maintained in a non-oxidizing atmosphere to a temperature of 1550° F. as a maximum, cooling it further and within a maximum time interval of two minutes

to dull red, then making the material into packs, and allowing the packs to cool in the air to atmospheric temperature.

In testimony whereof we have hereunto set our hands.

HENRY S. MARSH.  
RALF S. COCHRAN.

10

### DISCLAIMER

1,610,567.—*Henry S. Marsh and Ralf S. Cochran, Youngstown, Ohio. ANNEALING or SHEET STEEL.* Patent dated December 14, 1926. Disclaimer filed March 28, 1935, by the assignee, *Surface Combustion Corporation*.

Therefore, enters this disclaimer to any performance of the method recited in claim 2 of the said Letters Patent, except upon ordinary commercial steel, and with the result and effect of gaining relatively high ductility.  
[Official Gazette April 23, 1935.]

## DISCLAIMER

1,610,567.—*Henry S. Marsh and Ralf S. Cochran*, Youngstown, Ohio. ANNEALING OR SHEET STEEL. Patent dated December 14, 1926. Disclaimer filed March 28, 1935, by the assignee, *Surface Combustion Corporation*.

Therefore, enters this disclaimer to any performance of the method recited in claim 2 of the said Letters Patent, except upon ordinary commercial steel, and with the result and effect of gaining relatively high ductility.

[*Official Gazette April 23, 1935.*]